

# United States Patent

[19]

Harris

[11] 3,825,789

[45] \*July 23, 1974

[54] VACUUM ARC DEVICES WITH HARD,  
DUCTILE, FERROUS ELECTRODES3,281,563 10/1966 Waterton ..... 200/144 B  
3,551,622 12/1970 Takeuchi et al. ..... 200/144 B  
3,769,538 10/1973 Harris ..... 313/233[75] Inventor: **Lawson P. Harris**, Scotia, N.Y.[73] Assignee: **General Electric Company**,  
Schenectady, N.Y.[\*] Notice: The portion of the term of this  
patent subsequent to Oct. 30, 1990,  
has been disclaimed.[22] Filed: **June 29, 1973**[21] Appl. No.: **375,133**[52] U.S. Cl. .... **200/144 B**, 313/233, 313/311[51] Int. Cl. .... **H01h 1/02**, H01j 1/02

[58] Field of Search: .... 313/233, 311; 200/144 B

## [56] References Cited

## UNITED STATES PATENTS

1,582,330 4/1926 Brach ..... 313/311  
2,391,459 12/1945 Hensel ..... 313/311  
3,163,734 12/1964 Lee ..... 200/144 B

Primary Examiner—James W. Lawrence

Assistant Examiner—Wm. H. Punter

Attorney, Agent, or Firm—Jerome C. Squillaro; Joseph  
T. Cohen; Julius J. Zaskalicky

## [57] ABSTRACT

Vacuum arc devices utilized to protect electric circuit elements against very high transient currents and voltages and exhibiting high recovery voltage and high voltage holdoff strength include primary arc electrodes fabricated from hardenable ferrous material exhibiting high hardness, ductility, and high tensile strength. Such vacuum arc devices are superior to similar devices utilizing copper or cuprous alloy electrode materials because of increased mechanical strength and increased voltage holdoff strength and higher current interruption capacity.

14 Claims, 3 Drawing Figures



PATENTED JUL 23 1974

3,825,789

SHEET 1 OF 3

Fig. 1



PATENTED JUL 23 1974

3,825,789

SHEET 2 OF 3

Fig. 2



PATENTED JUL 23 1974

3,825,789

SHEET 3 OF 3



Fig. 3

## VACUUM ARC DEVICES WITH HARD, DUCTILE, FERROUS ELECTRODES

### RELATED INVENTIONS

This invention is related to the invention described and claimed in my co-pending application Ser. No. 236,278, filed Mar. 20, 1972, of which this application is a continuation-in-part the disclosure of which is incorporated herein by reference thereto.

### BACKGROUND OF THE INVENTION

The present invention relates to improved vacuum arc devices. More particularly, the invention relates to such improved devices as vacuum gaps, triggerable vacuum gaps, vacuum switches and the like.

In the art of vacuum arc devices, arcs are struck by the separation of a pair of arc electrodes or by the infusion of condensable conducting medium such as an electron-ion plasma into an evacuated chamber, generally evacuated to a pressure of at least  $10^{-5}$  Torr with a very high voltage applied across the arc electrodes. Ideally, once the arc has been struck, specie from the arc cathode is removed or boiled off therefrom to provide electron-ion plasma having a high density which forms the conducting medium between the arc electrodes carrying very high currents up to and including hundreds of thousands amperes of current for short times. In vacuum arc devices, the electrode material has a predetermined vapor pressure and, depending upon the value of vapor pressure evolves a quantity of conducting species so as to allow for a high current arc during a relatively short period of time as, for example, a portion of a half cycle of an alternating current voltage at 60 Hz frequency. Should this value be very low so that a too sparse quantity of conducting specie is evolved, the phenomenon known as "chopping" may occur. Chopping is a phenomenon that occurs due to vapor starvation and is characteristic of materials with too high a boiling point or too low a vapor pressure of the arc electrode materials. When chopping occurs, as a positive half-cycle of an alternating voltage approaches current zero and as the current begins to fall, current is suddenly extinguished, causing a high voltage transient to be reflected back into the system protected by the device, potentially causing damage, particularly in inductive circuits.

While the chopping phenomenon may be avoided readily by the provision of high vapor pressure materials as, for example, one or more of those materials set forth in U.S. Pat. Nos. 2,975,255 - Lafferty and 2,975,256 - Lee and Cobine, an over-plenteous supply of conducting specie may have deleterious effects. Thus, for example, when the current zero, alluded to above, is reached, the supply of conducting specie present can be too great such that the rate of condensation thereof and the recovery of a dielectric voltage holdoff strength may not occur at a sufficient rate to preclude a restrike of the arc when the opposite half-cycle of an alternating voltage is applied between the arc electrodes, particularly at high voltages.

In addition to the foregoing, soft arc electrode materials which generally have high vapor pressure tend to weld readily when joined together in switches and reclosers thus making the separation thereof on the next operation difficult, if not impossible.

Still another disadvantage of high vapor pressure materials as vacuum arc electrodes is that those materials tend to be mechanically soft and may readily be deformed or rapidly eroded by the boiling away of a too-plenteous supply of conduction specie during arcing.

On the other end of the spectrum, if the arc electrode material is of a much lower vapor pressure material, as for example molybdenum, tungsten, and other refractory metals which avoid the erosion and welding problems presented by high vapor pressure material, current chopping can occur. Even if current chopping does not occur, or is not of serious consequences, a limitation of usefulness under some circumstances is imposed by the thermionic emission characteristics of such refractory materials. Thus, for example, during a half cycle of alternating current at which a given arc electrode functions as an anode, anode spots tend to occur by the bunching of current footprints and portions of the anode electrode become exceptionally hot. 10 On the next half cycle, when the polarity of the arc electrodes is reversed, such a hotspot on a refractory material arc-cathode of, for example, molybdenum or tungsten, may function as an excellent thermionic emitter, thus causing thermionic emission of electrons from 15 the arc-cathode upon the application of the reverse bias voltage causing a restriking of the arc which cannot be tolerated.

Thus, the choice of arc electrode materials for vacuum arc devices is a tradeoff between conflicting requirements and must be made with due care.

Accordingly, it is an object of the present invention to provide vacuum arc devices possessing improved arc electrode materials which have ideal vapor pressure and boiling point characteristics so as to avoid current chopping or interruption failure due to excessive thermionic emission on one hand, or interruption failure or poor life due to excessive metal vapor evolution on the other hand.

Still another object of the invention is to provide vacuum arc devices possessing improved mechanical strength which facilitate high voltage recovery strength and higher current interruption than devices of the prior art.

Yet another object of the present invention is to provide improved vacuum arc devices suitable for holding off higher voltages, interrupting higher currents, operating with better electrical characteristics than devices of the prior art.

Yet another object of the present invention is to provide vacuum arc devices having arc electrode materials which are relatively inexpensive and which may be readily processed by conventional techniques for the production of high quality devices at relatively low cost.

### BRIEF DESCRIPTION OF THE INVENTION

Briefly stated, in accord with one embodiment of the present invention, vacuum arc devices in accord therewith include an hermetically evacuated envelope, evacuated to a pressure of  $10^{-5}$  Torr or less, and containing therein a pair of primary arc electrodes adapted to sustain a high voltage under non-arcing conditions and, under arcing conditions, to sustain a high current arc and to interrupt the same rapidly upon the cessation of current therethrough as, for example, by the occurrence of a normal current zero on an alternating current cycle. Such electrodes in accord with the invention

are fabricated of a gas-free, hardened, ductile, ferrous metal which exhibits all of the qualities of freedom from all gases and gas-forming impurities incompatible with such high vacuum, high hardness, reasonable ductility, and a characteristic of high voltage recovery strength and high rate of voltage recovery strength.

The novel features characteristic of the invention are set forth in the appended claims. The invention itself, together with further objects and advantages thereof, may best be understood by reference to the following detailed description taken in connection with the appended drawings in which:

FIG. 1 is a schematic, vertical, cross-sectional view of a vacuum arc device constructed in accord with the present invention;

FIG. 2 is a schematic, vertical, cross-sectional view of an alternative embodiment of a device constructed in accord with the present invention; and

FIG. 3 is a graph illustrating the voltage recovery characteristics of various electrode materials illustrating the advantages of devices constructed in accord with the present invention.

#### DETAILED DESCRIPTION OF THE INVENTION

In FIG. 1, a triggerable vacuum gap device represented generally as 10, comprises an hermetically sealed evacuable envelope 11 evacuated to a pressure of  $10^{-5}$  Torr or less. Envelope 11 comprises a cylindrical insulating sidewall member 12 supporting at respective ends thereof a pair of endwall members 13 and 14. Upper endwall member 13 is connected with cylindrical sidewall member 12 by a conventional insulator-to-metal seal flange 15 soldered, brazed, or otherwise affixed to endwall 13 and embedded in insulating sidewall 12. A similar insulator-to-metal seal flange 15 is used to connect in hermetic seal bottom endwall member 14 to cylindrical sidewall member 12. A pair of primary arc electrodes 17 and 18 defining an interelectrode gap 16 are respectively disposed in fixed mechanical and electrical conductive relationship with respective endwall members 13 and 14. Arc electrode member 17 is supported by an electrode support member 19 from endwall member 13 and electrode member 18 is supported from bottom endwall member 14 by an electrode support assembly 20. Arc electrode support 19 is comprised of a central core 21 of copper or cuprous alloy, for example, of high electrical conductivity which is abutted into and affixed with a good electrical conductive joint to arc electrode 17. Arc electrode 17 is fabricated from a gas-free, hard and ductile ferrous material, as is described with greater particularity herein-after. An arc support sheath member 22, also fabricated from a gas-free, hard, ductile, ferrous material may surround central core member 21. In like fashion, arc support assembly 20 comprises a cuprous or copper, for example, high electrical conductivity core member 23 which may be surrounded by a ferrous sheath member 24. Copper or cuprous core member 23 is embedded into ferrous arc electrode member 18 in good mechanical and electrically conductive joint, as is described hereinbefore with respect to arcelectrode support core 21. Additionally, a hollow bore 25 is made within arc electrode support member 23 and a trigger electrode assembly 26 containing a trigger anode 27 and a trigger gap 28 is disposed centrally within primary arc electrode member 18 to serve as a means for initiating an electric discharge between primary arc

electrode members 17 and 18 by the application of an electric pulse through trigger anode lead 28 to trigger anode 27 to cause a breakdown of trigger gap 28 and the infusion of electron ion plasma into primary arcing gap 16. Trigger electrode 26 is shown herein without detail. Details of suitable trigger assemblies may, for example, be found in U.S. Pat. Nos. 3,087,092, 3,465,192 and 3,465,205.

A shield assembly 31 which may, for example, comprise a large primary shield member 32 in the form of a cylindrical member depending from upper endwall member 13 and extending approximately two-thirds to three-quarters of the distance between endwall members 13 and 14 encompassing the area surrounding the arc gap 12 and a second cylindrical shield member 33 upwardly depending from lower endwall member 14 and terminating short of shield member 32 leaving a gap 35 by a distance which is large as compared with arcing gap 16 surrounds the arc electrodes and protects the insulating integrity of insulating sidewall 12. A deflector shield member 34 in the form of a foreshortened truncated conical member depends from lower arc electrode support assembly 20 and has an angle with respect to the normal to the axis of the arc electrode support members which is directed to a point along shield member 32 above gap 35, such that conduction species emanated from arcing gap 16 is deflected by shield member 34 to shield member 32 without allowing a line-of-sight passage to gap 35 from arcing gap 12 such that conduction species emanating from an arc between the primary arc electrodes are deflected to shield member 32 short of gap 35. A distance between shield members 34 and 32, like the distance between shield members 32 and 33, is large as compared with the interelectrode gap 16. While the illustrated shield arrangement is shown by way of example, it should be appreciated that other shield arrangements may be utilized in devices in accord with the invention.

In operation, a high voltage of, for example, 30 kilovolts, is placed across arc electrode support assemblies 19 and 20 as, for example by connecting an appropriate lug at screw connector 36 and a similar connector (not shown) on the end of arc electrode support member 20. Such high voltage may be across an electrical device as, for example, a transformer or a capacitor which is to be protected against voltage transients and the vacuum gap and it may be used to short such transients by applying a pulse as, for example, by means of a voltage source represented schematically by battery and switch 37, between trigger anode lead 29 and base member 13 which is electrically connected to arc electrode 18. Alternatively, a sample of the voltage between the primary arc electrodes may be applied between the trigger anode and arc electrode 18. When such a trigger voltage is applied, trigger gap 28 breaks down and an electron ion pulse is injected into gap 12 instituting the initiation of an electric arc which is thereupon carried between arc electrodes 17 and 18 until the occurrence of current zero, at which time the arc is extinguished. Alternatively, the gap 16 may itself breakdown and no trigger electrode assembly need be included.

As is indicated hereinbefore, in the long and tortuous development of vacuum arc devices, those skilled in the art have worked to provide vacuum arc electrodes of materials having intermediate vapor pressures and boiling points to provide arc conduction specie for such

devices. A necessary criterion for such arc electrode material is that it may be vacuum processed to remove therefrom all sorbed gases or gas-forming constituents which, upon the formation of a high current arc, can cause the evolution of gaseous contaminants which would permanently affect the maintenance of a steady-state equilibrium pressure of the order of  $10^{-5}$  Torr or less. A further consideration has been the seeking of arcing material which exhibits good chopping characteristics, namely, the ability to hold the current as a cycle of current alternation upon which an arc has been struck approaches zero without having the current abruptly terminated from a relatively high value to zero with the creation of a high voltage transient. For these reasons, among others, the art has concentrated upon the use of copper and cuprous alloys of vacuum arc devices.

Furthermore, it has been an unwritten folklore that the use of any ferromagnetic materials in arcing electrodes in vacuum arc devices would result in unpredictable and deleterious magnetic effects and is, therefore, to be avoided. Additionally, such materials have generally been avoided in devices in which any substantial steady-state current is to be conducted because of the lesser electrical conductivity of ferrous materials than cuprous materials. For these reasons, innovators working with arcing materials have generally avoided ferrous materials. I have found, however, that the problem of the electrical conductivity of ferrous materials is not as serious as had previously been considered, provided that the ferrous material is used under certain circumstances. Thus, for example, in a vacuum arc device which does not carry a steady-state current, but only a fault current during arcing, as the device of FIG. 1, I have found, unexpectedly, that the electrical conductivity of certain ferrous materials, as described herein, after in accord with the present invention, is entirely adequate to sustain the current conduction during the relatively short arcing periods that high currents are carried. Thus, I have found that high currents of the order of kiloampere arcs and arcing times of the order of one cycle of power frequency alternating current do not provide any problems, even considering the higher electrical resistivity of ferrous materials than copper, and like materials. This is true at this time because present vacuum arc device technology has overcome the early (e.g., 1950-1960) problems relating to problems of sufficient arcing species to sustain an arc, avoiding unacceptable chopping currents and avoiding the formation of destructive arc footprints, particularly anode spots. The present problems facing innovators in the vacuum arc art relate largely to extending the magnitude of voltage which may be safely impressed between arcing members and increasing the currents which may be interrupted and thereby terminated. This is particularly true in the case of vacuum gap devices wherein a fixed gap exists and no steady-state electrical conduction of the main current is provided, but current is conducted only for a very short time during arcing under fault voltage conditions.

Since the chopping characteristics of iron and of ferrous materials in general are compatible with vacuum arc use, and so long as ferrous materials are not used as extended conductors for steady-state conduction of high currents, there is thus no electrical disadvantage to their proper use in vacuum arc devices. I find, however, that there are decided advantages. Thus, for ex-

ample, the degassification of ferrous materials is relatively simple. Initial degassification of the bulk material may be provided by vacuum-melting, a technique of relatively recent commercial use, not available until recently for vacuum arc devices or the fabrication of ferrous electrodes for use therein. Such vacuum-melting, particularly of the consumable electrode type vacuum melting wherein each portion of a ferrous bar from which the finally utilized ferrous electrode is formed, is at one point the arcing point of a vacuum arc and each portion of the arc electrode source material is melted under vacuum conditions to cause the removal of all gas and gas-forming constituents before formation of the electrode is an inexpensive method of preparing highly gas-free metal for vacuum arc electrodes. Once the electrodes have been formed from such material, the surface degassification of adsorbed gaseous material is quite simple. Ferrous materials, as with cuprous materials, may be degassified of adsorbed gases merely by assembling them in the vacuum arc device and during normal bakeout, subjecting them to the temperature and time of bakeout necessary to degassify the other materials in the device. Due to their high temperature characteristics, such bakeout temperatures are not limited thereby.

Of greatest importance and bearing upon the utility and advantages of ferrous arc electrode materials in accord with the present invention, I have found that the use of hard and ductile gas-free arc electrode materials results in the attainment of a high dielectric recovery characteristic and high electrical breakdown strength as well as a more rapid rate of recovery of such high electrical breakdown strength than any cuprous material. This characteristic greatly facilitates a substantial increase in voltage rating of devices in accord with the invention as compared with prior art devices utilizing conventional electrode materials.

While numerous ferrous materials are useful in the production of vacuum arc devices in accord with the present invention, I find that certain hardenable steels having martensitic grain structure and certain precipitated inclusions are particularly useful. Many of these steels may be machined while relatively soft in condition and then heat-treated to cause an increase in hardness and yield strength and are ideally suited for devices in accord with the present invention.

One general grouping of such steels is well known and generally identified as "age hardening" or "precipitation hardening" steels. In general, these steels are martensitic steels obtained by quenching rapidly an austenitic steel to obtain dispersion of impurities and small grain size. Hardening is effectuated by the presence of impurities, which also contribute to the necessary ductility. The hardening may result from a heat treatment generally performed at a relatively low temperature (as compared with the temperature of the original quenching), as for example between 900°-1,000°F. Some such steels are iron-nickel maraging steels (generally containing also minor quantities of molybdenum and cobalt, and sometimes titanium) with from 15 to 30 weight percent nickel. Some such steels are described in an article entitled "18 percent Nickel Maraging Steel" by Decker, Eash and Goldman, published in the Transactions of the ASM, pp. 58-76, 1962. Certain specific maraging steels which have been found suitable for use in the invention are available from Vanadium Alloy Steel Co., Latrobe, Pennsylva-

nia, and are described in a brochure copyrighted by that firm in 1966 entitled VASCOMAX 200-250-300-350 which brochure lists many specific compositions of suitable maraging steels.

Maraging steels are normally manufactured by vacuum melting practices and are relatively free of dissolved gases as commercial steels go. Developmental tests have verified that the gas content of these steels is acceptable for use in arc electrodes in vacuum arc devices. As purchased commercially, maraging steels may typically have a hardness of approximately 30 Rockwell C and exhibit a yield strength of approximately 100,000 psi, approximately six times that of copper. In this condition the steels are, nevertheless, readily machinable, much more so than copper. After machining, forming and other preparation for assembly into the devices of the invention, the maraging steels may be hardened by a high-temperature aging treatment, the temperature and time of which may be varied compatibly to achieve the useful result. Thus, for example, a typical 30 Rockwell C 100,000 psi maraging steel, after treatment at 520°C for approximately three hours, exhibits a hardness of 54 Rockwell C and a yield strength in excess of 250,000 psi with remarkably high ductility in excess of 10 percent of 2 inches length and standard cross section. Such characteristics are uniquely adapted for the formation of electrode assemblies in vacuum arc devices since the bakeout time of such devices may be sufficient to cause appropriate hardening of a maraging steel. Thus, for example, I have constructed vacuum devices in accord with the present invention utilizing a particular maraging steel known as VASCOMAX 300 CVM to form arc-electrode members exhibiting the foregoing mechanical characteristics. In one illustrative instance, VASCOMAX 300 CVM maraging steel having a 30 Rockwell C hardness was machined to provide arc electrode members of vacuum arc electrode assemblies in accord with the present invention, assembled, and the device was baked-out for 24 hours at 550°C. After such treatment, the steel was found to exhibit a hardness of approximately 41 Rockwell C and a corresponding yield strength of 150,000 psi, at least ten times stronger than conventional vacuum processed OFHC copper generally utilized in such devices, and a ductility in excess of 10 percent. As is mentioned hereinbefore, for short term arcing characteristics, the steels of the invention are comparable to copper insofar as arcing current-carrying capacity is concerned. Developmental tests of VASCOMAX 300 steel utilized as described herein have shown an ability to carry without deleterious effect a current density of approximately 225 amperes/cm<sup>2</sup> over the surface thereof for a half cycle of arcing, which is equal to or better than the same value as may be carried by copper electrodes.

Other hardened or hardenable steels from which ferrous arc-electrodes for use in devices in accord with the invention are made, include precipitation-hardened stainless steels such as those set forth on pages 81 and 83 of the "1972 Materials Selector" published by Materials Engineering Journal, Stamford, Connecticut. Such precipitation-hardened stainless steels, no one of which is unique in desirable properties as used herein, usually contain low carbon, high nickel and chromium and minor precipitates of other elements. They are generally hard, having tensile strengths in excess of 150,000 and usually in excess of 200,000 psi, are easily

outgassed and have ductility of the order of 10 percent elongation of standard 2 inches long standard test section. Many other precipitation-hardened stainless, austenitic and martensitic steels may be found.

One specific precipitation-hardened stainless steel possessing characteristics ideally adapted for use in devices in accord with the invention is identified as "Carpenter Custom 455" and is available from Carpenter Technology Corporation, Reading, Pennsylvania. This steel contains approximately 12 percent chromium, 8.5 percent nickel, 1.2 percent titanium, 2.25 percent copper, less than 1 percent each of carbon, manganese and columbium, balance iron. Its tensile strength is in excess of 225,000 psi, readily outgassed and has high ductility as represented by a 5-10 percent elongation in a standard 2 inches long test section of standard cross section.

Still another class of uniquely adapted hardened ferrous materials or alloys well adapted for use in devices in accord with the invention are the so-called TRIP steels (Transformation Induced Plasticity). Such steels are normally austenitic, but their composition places them near the phase line so that warm working causes a transformation to martensite under stress at service temperatures. A description of TRIP steels may be found in an article appearing in preprint No.-UCRL 18609 (Lawrence Radiation Laboratory), University of California, November 1968, by W. W. Gerberich and entitled "Metastable Austenitic Steels with Ultrahigh Strength and Toughness." See also TRANS. ASM 60, 252 (1967), "The Enhancement of Ductility in High Strength Steels" by Zackey et al.

In general, another class of ferrous alloy materials which may be utilized in accord with the present invention is that of carbon alloy steels. These steels differ from maraging steels, and other hardenable steels which are often soft after a quench from a high temperature in excess of 1500°F and hardened by later exposure to intermediate temperatures of the order of 900°F-1200°F that correspond reasonably well to bakeout temperatures of vacuum arc devices in accord with the present invention. Carbon alloy steels, on the other hand, as is epitomized for example by VASCO-JET 1000 CVM, a carbon alloy steel available from Vanadium Alloy Steel Co., Latrobe, Pennsylvania, and comprising approximately 0.40 percent carbon, 5.0 percent chromium, 1.3 percent molybdenum, 0.5 percent vanadium, the remainder iron, are hardened by a quench from a high temperature (1,800°-1,900°F for VASCOJET 1000) and later tempered to slightly decrease the hardness and increase the ductility by exposure to intermediate temperatures such as those utilized in the bakeout of vacuum arc devices in accord with the present invention.

I am aware that ferrous materials of largely unspecified characteristics have been used in vacuum arc devices previously. Thus, U.S. Pat. No. 1,582,330 issued Apr. 27, 1926 on an application filed May 19, 1919 by L.S. Brach, wherein the use of nickel steel of unspecified hardness, ductility and other characteristics other than that the nickel steel does not, it is stated, emit gases, has been utilized in a lightning arrester, as gap electrode therefor. The teaching of the Brach patent does not bear a substantial relation to the use of the specific hard, ductile highly pure and gas-free arc electrodes disclosed and claimed in accord with the present invention since the state-of-the-art in 1919, insofar as

vacuum is concerned, was very crude and in no way advanced to the point where vacuum arc devices as considered in the present era were feasible. Thus, for example, a vacuum of  $10^{-5}$  Torr was not obtainable in 1919 for devices of this nature at the time the Brach application was filed. Similarly, the nickel steel disclosed by Brach is of unspecified hardness and ductility and as is set forth hereinafter, cannot be assumed to have the unique characteristics of hardness and ductility associated with the unique high dielectric strength and high rate of recovery strength of the vacuum arc electrodes in accord with the present invention.

Not all ferrous materials exhibit the same characteristics of voltage recovery strength and rate of voltage recovery strength, which are essential in accord with the present invention. I am further aware that U.S. Pat. 3,038,980 issued June 12, 1962 on an application filed Dec. 17, 1959 to T. H. Lee makes the generalized statement that "the property of a metal that appears to be most predominant in determining the voltage at which a breakdown between electrodes of such metal will occur is its modulus of elasticity in tension, i.e., Young's Modulus". While superficially it may seem that Young's Modulus of Elasticity is related to the hardness and/or ductility of devices in accord with the present invention, it should be pointed out that Young's Modulus of Elasticity is an indication of the tensile strength of the material within the elastic range and is generally achieved by computing the ratio of stress to strain during elastic deformation. Ductility, on the other hand, is related to plastic deformation, which characteristics are entirely unrelated. Young's Modulus is not an indication of the hardness of a material. Furthermore, Young's Modulus of Elasticity is essentially the same for all irons and steels, whereas, as may be found by reference to FIG. 3 which will be discussed hereinafter, the voltage recovery strength and rate of voltage recovery strength which are critical to the selection of ferrous arc electrode materials in accord with the present invention, vary substantially among ferrous materials which meet the criteria of hardness and ductility and gas freedom, as set forth herein.

The importance of ductility in arc-electrodes of vacuum arc devices in accord with the invention cannot be stressed too heavily. The enormous shocks caused by the electromagnetic forces of kilo-ampere arc can deform strong arc electrode structures. If the structures are merely made hard, they may be brittle, and when stressed may crack or break. The advantages of the invention are only achieved when the hard ferrous material utilized is sufficiently ductile, as is defined herein, to withstand the shocks and absorb the same without deforming or shattering.

It is apparent to those skilled in the art that with the opening of the possibilities of hard, ductile, ferrous alloys such as maraging, precipitation-hardened, TRIP, and carbon steels which are capable of having their crystal structure grain size and other metallurgical characteristics altered by treatment at temperatures which may correspond with acceptable temperatures for the bakeout of vacuum arc devices in accord with the present invention, that this invention may be practiced with numerous such steels, many of which may provide the increased strength, hardness and ductility which are desirable and consistent with the attainment of more stable vacuum arc structures for the attainment of higher currentcarrying capabilities and greater

dielectric strength. Accordingly, it is well within the contemplation of those skilled in the metallurgical arts to apply the teachings of the present invention to the use of many unenumerated ferrous alloys for the provision of improved vacuum arc devices.

As used herein, and in the appended claims, the terms "hardness", "hard", and the like, are intended to connote a tensile strength in excess of 100,000 psi and preferably in excess of 150,000 psi and a Rockwell C value of at least approximately 30 and preferably at least approximately 40. As used herein, the terms "high ductility", "ductile" and the like are meant to connote a ductility as evidenced by a percentage elongation of a standard 2 inches long sample of standard (ASTM) cross section of at least 5 percent and preferably 10 percent. All percentages of compositions are expressed in weight percent.

FIG. 2 of the drawing illustrates a vacuum switch constructed in accord with the present invention. In FIG. 2, like elements to those of FIG. 1 are identified with like numerals. In FIG. 2, as in FIG. 1, envelope 11 of vacuum switch 50 comprises upper and lower endplates 13 and 14, respectively, separated by cylindrical insulating endwall member 12. A pair of arc electrode members 17 and 18 defining an arcing gap 16 therebetween are supported respectively from endwall members 13 and 14 by arc electrode support assemblies 19 and 20 respectively. Arc support assemblies 19 and 20 are both comprised of a cuprous inner core 21 and 23 respectively which may be surrounded by a ferrous cladding member 22 and 24 respectively. The cuprous core members 21 and 23 are electrically and mechanically affixed with low resistance connection to arc electrodes 17 and 18 respectively. A copper-bismuth or copper-beryllium alloy, for example, arcing button 20 is inserted into arc electrode 18 primarily to prevent welding between like material arc electrodes 17 and 18. The presence of a low vapor pressure "button" in arc electrode 18 does not detract from the dielectric recovery strength and breakdown strength characteristics obtained due to the use of ferrous electrodes in devices in accord with the invention. Thus, the small size of button 20 and its central location, in view of the known electromagnetic tendency of an arc between two electrodes to propagate transversely and to seek the edges or corners thereof rapidly removes the arc from the central button so that its presence has essentially no effect on the voltage recovery strength and rate of recovery thereof of devices in accord with the invention.

Arc electrode support member 20 is reciprocally movable so as to move from a first circuit closed position in which it is in contact with fixed arc electrode 17 to an open circuit position in which it is separated from arc electrode 17 by gap 16. Reciprocal motion of arc support 20 is achieved by means of bellows member 40 which is affixed at one end thereof by flange 41 to the exterior of lower endwall 14 and at the other end thereof by flange member 42, which is affixed to the surface of reciprocable arc support member 20. Bellows assembly 40 is in hermetic seal with endwall member 14 and arc support assembly 20 so as to provide means for separating arc electrodes 17 and 18 while at the same time maintaining the necessary high vacuum within switch envelope 11. An equipotential high current conducting strap of a flexible braided conductor, preferably copper or a cuprous alloy, provides for good

electrical conduction between reciprocable assembly 20 and endwall 14 and is appropriately affixed thereto.

In operation, vacuum switch 20 is connected in circuit with a circuit element to be protected as, for example, a transformer or motor, and is normally connected in line with a current conduction path by means of connector 44 on arc electrode support member assembly 19 and a similar connection (not shown) on support assembly 20 or, alternatively, one affixed to lower endwall member 14. Steady-state conduction of electric current is essentially through the cuprous cores 21 and 23 of arc support members 19 and 20, with a minimal length of conduction path through ferrous material of arc electrodes 17 and 18, thus achieving the desirable electrical conductive characteristics of copper or cuprous materials together with the advantageous dielectric recovery voltage strength of the ferrous arc electrode materials in accord with the present invention. Upon occurrence of a voltage or current fault, requiring separation of the arc electrodes to protect the circuit or circuit elements associated therewith, a signal indicative of the fault actuates a conventional circuit breaker actuating mechanism (not shown) to cause arc electrode support assembly 20 to be reciprocably movable downward, removing arc electrode 18 from contact with fixed arc electrode 17 and causing the initiating of a high current arc to be struck therebetween. Thereafter, conduction of current through the high current arc and extinction thereof are essentially the same as in accord with the mode of operation of the triggerable vacuum arc device of FIG. 1 of the drawing. The device of FIG. 2 may be modified to form a triggerable switch by adding a trigger electrode assembly to one primary arc-electrode structure as is done in FIG. 1. Such a device is in a normally open position and is triggered to strike an arc.

As is stated hereinbefore, yet another unexpected advantage of devices in accord with the present invention is the discovery of a unique dielectric recovery strength characteristic of ferrous arc electrodes of the ductile, hardenable steels utilized in devices of the invention. FIG. 3 of the drawing illustrates a typical plot of recovery strength in volts plotted as a function of time after arcing of gas-free arc electrodes of a specific configuration following a 250 ampere shaped current pulse utilized in vacuum arc devices, as in the present invention, fabricated from different electrode materials tested under identical test conditions. In each instance, the voltage in kilovolts between the electrodes starts from a zero value and rises to a breakdown value, the average of which is generally denominated as the "recovery strength". Thus, two important characteristics are present. First, the rate of recovery in kilovolts per microsecond and the recovery strength in kilovolts (KV). In FIG. 3, curve A represents the recovery strength curve for copper electrodes. Curve B represents the recovery strength curve for beryllium electrodes. Curve C represents the recovery strength curve for electrodes made of two different steels typical of the hardened ductile steels in accord with the present invention, both of which have essentially the same recovery strength characteristics. These steels are VASCOMAX 200 and VASCOJET 1,000. Curve D represents the recovery strength characteristic of 304-type stainless steel, a readily available, commonly used, stainless steel, often

found as shield materials and other instrumentalities in circuit breakers and such devices.

As is set forth hereinbefore, all ferrous materials are not suitable for vacuum arc devices in accord with the present invention. Thus, Curve D, representative of the recovery strength characteristic of type 304 stainless steel, exhibits a recovery rate of approximately 8 to 10 kilovolts per microsecond as compared with the recovery rate of approximately 15 KV per microsecond shown by Curve C, and saturates at a value of approximately 70 kilovolts. Copper, on the other hand, shows both a slower recovery strength than that of the steels in accord with the present invention and saturates at a very low value of voltage, namely, 37 kilovolts. While this is not consistent with the curves shown in my above-identified copending application wherein it was stated that copper electrodes show essentially the same recovery rate of hard, ductile steels, later, more precise test data indicates the herein described added advantage in recovery rate of hard, ductile steel electrodes to be a more representative value. Beryllium, although exhibiting a very rapid rate of recovery strength, is inferior to the steels in accord with the present invention in that it saturates at approximately 60 kilovolts.

Thus, from a consideration of curves of FIG. 3, it may be seen that the electrodes fabricated from hard, ductile, gas-free steels in accord with the present invention make devices fabricated in accord with the present invention quite superior to those utilizing copper in that the recovery rate is higher and the saturation voltage holdoff strength is almost three times as great. Ordinary type 304 stainless steel shows both a lower recovery rate and a saturation value which is approximately 60 percent that of steel ferrous materials in accord with the present invention. It is, therefore, apparent that great utility may be found in the use of the hardened, ductile, gas-free, ferrous materials in accord with this invention in the fabrication of vacuum arc devices.

Thus, it is readily apparent that the unique advantages found in electrodes made of hard, ductile, gas-free, ferrous materials, as set forth herein, are not characteristic of electrodes of ferrous materials, per se, particularly alloy steels such as nickel steels, noting for example the inferior performance of electrodes made of 304 stainless steel which contains approximately 18 percent chromium, 8 percent nickel and the balance iron. All of the electrodes, the characteristics of which are illustrated graphically in FIG. 3, were similarly gas-free so that although the devices in accord with the present invention must contain electrodes which satisfy the gas-free criteria set forth hereinbefore, the subnormal performance of type 304 stainless steel electrodes, as is evidenced by the graph of FIG. 3, is not to be attributed to superior or inferior gas-freedom. Rather, as is set forth hereinbefore, the unique advantages of electrodes in accord with the invention, and devices in accord with the invention using such electrodes, is related to the unique combination of hardness and ductility found in hardenable steels, such as maraging steels, TRIP steels, carbon alloy steels, and precipitation-harden steels. Similarly, all of the steels used in electrodes in accord with the present invention are found to have significant proportion of impurities therein which make it possible for the grain structure thereof to be susceptible of the appropriate hardening under the particular characteristic and manipulative processes whereby the hardening of the unique steels uti-

lized in electrodes in accord with the present invention is accomplished.

In general, in addition to the steels set forth herein, other vacuum-refined steels containing nickel, chromium, and often titanium, and other such similar transition metals, are sufficiently hard, ductile, and may be readily rendered sufficiently gas-free as to be uniquely adapted to possess the highly desirable hardening characteristics which optimize devices utilizing such ferrous arc electrode assemblies in accord with the present invention.

Devices constructed in accord with the present invention have been operated repeatedly to hold off 100,000 volts in open circuit position. Switch devices in accord with the invention have, in closed circuit position, routinely successfully carried 33,000 amperes peak current. This current has been interrupted successfully by causing an arc to be struck which exhibits approximately a 50 volt drop and which has been extinguished at a first occurring current zero with no noticeable deleterious effects to the arc electrodes, and such arc has been extinguished and the applied voltage has failed to restrike on the next voltage half cycle.

While certain characteristics of the materials utilized in devices in accord with the invention are disclosed and claimed in my aforementioned co-pending application, it has, since the filing thereof, been discovered that certain other characteristics thereof are important and that my invention is broader in scope than the specific configuration of arc electrodes illustrated therein. Accordingly, the appended claims set forth in true depth and scope the invention disclosed herein. It is, therefore, my intention to cover by the appended claims all modifications and changes of the herein-disclosed embodiments as fall within the true spirit and scope of the foregoing disclosure.

What I claim as new and desire to secure by Letters Patent of the United States is:

1. A vacuum arc device adapted to carry high currents in one operative state and to hold off high voltages in another operative state and comprising:  
 a. an hermetically-sealed envelope evacuated to a pressure of  $10^{-5}$  Torr or less;  
 b. a pair of arc electrode assemblies disposed within said envelope and adapted to define therebetween an interelectrode gap and to sustain therebetween a high current arc which is sustained by conduction specie derived from said arc-electrodes;  
 c. said electrode assemblies comprising ferrous material having a hardness as evidenced by a Rockwell C hardness of at least 30, a yield strength of at least 100,000 psi, and a ductility as evidenced by at least a 5 percent elongation of a standard 2 inches long sample of standard ductility test cross-section and having a substantial freedom of sorbed gases and gas-forming impurities therein so as to withstand arcing current densities of approximately 200 amperes/cm<sup>2</sup> for a half-cycle of power-alternating

voltage without the emission of any substantial quantity of gaseous material inconsistent with continued maintenance of said low pressure after having been arced thereby.

- 5     d. shield means surrounding said arc electrode members to confine arcing specie to the interior thereof; and
- 10    e. means connecting said arc electrode assemblies in circuit with an electric load.
- 15    2. The device of claim 1 wherein each of said ferrous electrode assemblies is a vacuum-melted steel.
- 20    3. The device of claim 2 wherein said ferrous electrode assemblies are fabricated from hardened steel having a Rockwell C hardness in excess of 40, a yield strength in excess of approximately 150,000 psi, and a ductility corresponding to an elongation of at least approximately 10 percent of a 2 inches long standard cross section test sample.
- 25    4. The device of claim 2 wherein said ferrous assemblies are fabricated of age-hardened steel which increases in hardness and yield strength during vacuum bakeout cycles used to fabricate vacuum arc devices.
- 30    5. The device of claim 2 wherein said ferrous metal is precipitation-hardened.
- 35    6. The device of claim 4 wherein said bakeout temperatures are of the order of 900°-1,200°F and are utilized for periods of from 5-24 hours.
- 40    7. The device of claim 2 wherein said ferrous material is a transformation induced plasticity steel.
- 45    8. The device of claim 2 wherein said ferrous material is a temperature-hardened maraging steel.
- 50    9. The device of claim 3 wherein said ferrous material is temperature-hardened carbon alloy steel having from 0.2 to 0.6 weight percent carbon therein.
- 55    10. The device of claim 2 wherein the device further includes means for establishing an electric arc between said arc electrode assemblies by establishing an electron-ion plasma therebetween.
- 60    11. The device of claim 10 wherein said device is a triggerable vacuum gap device and the means for supplying an electron-ion plasma therein is a trigger electrode assembly.
- 65    12. The device of claim 10 wherein the device is a vacuum switch and said arc-electrodes are each supported upon a highly electrically conductive support member which is secured in low resistive contact with said ferrous arc-electrode.
- 70    13. The device of claim 12 wherein said electrode support members are surrounded by a sheath of hard, ductile, ferrous material.
- 75    14. The device of claim 3 wherein said ferrous assemblies are fabricated of a heat treatable steel which increases in ductility during vacuum bakeout cycles used to fabricate vacuum arc devices of the order of 500°-600°C.

\* \* \* \* \*